# EUROPEAN PATENT SPECIFICATION

(11) **EP 2 257 439 B1**
(45) Date of publication and mention of the grant of the patent: **24.07.2013**
(21) Application number: 09720285.7
(22) Date of filing: 10.03.2009
(51) Int. Cl.: B41N 7/04

(54) **USE OF A ROLLER BODY HAVING A ROLLER COATING FOR IMPROVED INK-WATER-EMULSION FORMATION IN PRINTING UNITS OF WET OFFSET MACHINES**
VERWENDUNG EINES WALZENKÖRPERS MIT WALZENBESCHICHTUNG FÜR VERBESSERTE TINTE-WASSER-EMULSIONSBILDUNG BEI DRUCKWERKEN VON NASSOFFSETDRUCKMASCHINEN
UTILISATION D'UN CORPS DE CYLINDRE POSSÉDANT UN REVÊTEMENT DE CYLINDRE POUR AMÉLIORER LA FORMATION DE L ÉMULSION ENCRE/EAU DES UNITÉS D IMPRESSION DES MACHINES OFFSET HUMIDES

(30) Priority: 13.03.2008 DE 102008014034
(43) Date of publication of application: 08.12.2010
(73) Proprietor: Coatec Gesellschaft Für Oberflächenveredelung Mbh, 36381 Schlüchtern (DE)
(72) Inventor: Johner, Gerhard, 63751 Gelnhausen (DE); Kirst, Markus, 64572 Büttelborn (DE)
(74) Representative: Schwan - Schwan - Schorer
(86) International application number: PCT/EP2009/052752
(87) International publication number: WO 2009/112471

(56) References cited:
- EP-A- 0 412 219
- WO-A-00/49301
- GB-A- 2 269 136
- US-A- 5 235 747
- US-A- 5 317 966
- US-A1- 2002 187 292
- US-B1- 6 290 633

## Description

The invention relates to the use of roller bodies made of steel, aluminium or carbon fibre reinforced plastic material in printing units of wet offset machines, having a roller coating, the objective of which is to guarantee the formation of a stable ink-water-emulsion.

According to the prior art such roller bodies are provided with matted chromium coatings (see roller assembly according to Fig. 1) or with RILSAN® coatings (usual product name in offset machines for coatings from the group of polyamides, see roller assembly according to Fig. 2). The latter coatings are regarded as lipophilic and wear-resistant and very often show a very smooth surface, in particular if the printing unit operates with highly-pigmented ink or even zinc white including titanium dioxide pigments. Already after a short operation, highly pigmented inks very often have the effect, that even layers of matted chromium are heavily smoothened and lose the desired surface roughness. Neither a smoothened coating of matted chromium nor a smooth RILSAN® coating are able to form in a sufficient quantity the stabile ink-water-emulsion which is necessary for the printing process, with the consequence, that according to the prior art emulsification aids in the form of isopropyl alcohol and/or tenside-containing additive are added to the fountain solution. These additional measures are as such undesirable, because they are cost-increasing and damaging to the environment (isopropyl alcohol is regarded as damaging the atmosphere and is a volatile organic compound). Moreover, in the practice of low-isopropyl or isopropyl-free printing it turned out that partly not before weeks of operation of the printing unit, an increase in the concentration of the tenside-containing additives leads to an overturning of the printing process, because there is no longer a "water-in-ink-ernulsion", but rather an "ink-in-water-emulsion"; the latter, of course, wets not only the ink-cantaining zones on the printing plate, but also the water-containing zones, so that not print pattern is produced on the paper to be printed, but only an uncontrolled inking.

GB 2 269136 A discloses a dampening-unit roller of a printing machine with an improved hydrophile effects by adding to the dampening medium only little alcohol or none at all. Such hydrophile properties are obtained with a coating having a surface roughness which is smaller than 5 µm, In particular smaller than 1 µm.

The invention aims at providing coated roller bodies of steel, aluminium or fibre reinforced plastic material, which in wet offset machines are in direct contact to the dampening form roller and which serve the formation of a stable ink-water-emulsion, which coated roller bodies have a wear-resistant surface the topography of which does not change during the printing machine operation even if inks with many pigments which may have very abrasive effects are processed, and which coated roller bodies permanently maintain a sufficiently high roughness. Furthermore, a relatively simple and cost-effective method for the manufacturing of such coated roller bodies is described. The objective of the invention is solved according to claim 1.

In particular, the roller bodies of steel, aluminium or fibre reinforced plastic materials to be coated, which in wet offset machines are in direct contact with the dampening form roller, are provided with a porous coating made of highly wear-resistant oxide ceramics such as, for example, Al₂O₃, Cr₂O₃, TiO₂, SiO₂ or ZrO₂ or mixtures thereof, or made of wear-resistant hard metal such as for example, WC/Co, Cr₃C₂/NiCr, NiCrBSi, WC/Ni, TiC/Ni, molybdenum, chromium etc., which coating preferably is applied by means of a thermal spraying method and is subsequently ground to size, so that pores in the matrix of the layer are opened.

The surfaces produced in this process preferably show roughnesses of 1.0 µm < R_{z} < 500 µm, in particular R_{z} = 5 µm to 25 µm. The thicknesses of the porous coatings according to the invention preferably range from 25 µm to 2000 µm, preferably at about 150 µm. The porous coating according to the present invention made of oxide ceramics or hard metal does not have to be applied by thermal spraying, but may also be applied by means of coating methods such as PVD (Physical Vapour Deposition), CVD (Chemical Vapour Deposition), sintering, enamelling, hot isostatic pressing, electroplating, explosion cladding, build up welding, build up brazing, adhesion methods or reactive processes. If the roller body to be coated is made of fibre reinforced plastic material and the coating process involves a thermal spraying process, it preferably has to be taken into account that a circumferential velocity of at least 0.2 m/s is observed and cooling processes are applied, which keep the fibre reinforced plastic material below 200°C, because otherwise a delamination may occur.

In Fig. 1 an emulsification aid in the form of a distributor cylinder R designed in the above-described manner is shown, which is positioned below a dampening form roller 1 of a wet offset machine. As is known, an ink-water-emulsion is applied onto a plate cylinder by the dampening form roller 1.

Fig. 2 shows an emulsification aid in the form of a porously coated tandem roller T on the dampening form roller 1.

## Claims

1. Use of a roller body for improved ink-water-emulsion formation in printing units of wet offset machines, which roller body is in direct contact with the dampening form roller of the printing units of wet offset machines, the roller body being made of steel, aluminium or carbon fibre reinforced plastic material, **characterized by** a coating of the roller body being made of highly wear-resistant oxide ceramics or of wear-resistant hard metal, wherein pores which are open towards the circumferential surface of the roller body, are provided in the layer matrix of the coating, and wherein the porous coating has a surface roughness R_{z} of 5 µm to 25 µm.

2. Use as claimed in claim 1, **characterized in that** the porous coating consists of Al₂O₃, Cr₂O₃, TiO₂, SiO₂ or ZrO₂ or of mixtures thereof.

3. Use as claimed in claim 1, **characterized in that** the porous coating consists of WC/Co, Cr₃C₂/NiCr, NiCrBSi, WC/Ni, TiC/Ni, molybdenum, chromium or of mixtures thexeof.

4. Use as claimed in any one of the preceding claims, **characterized in that** the porous coating has a thicknesses of 25 µm to 2000 µm, preferably a thicknesses of about 150 µm.

## Patentansprüche

1. Verwendung eines Walzenkörpers zur verbesserten Farb-Wasser-Emulsionsbildung in Druckwerken von Nassoffsetmaschinen, wobei der Walzenkörper in direktem Kontakt zur Feuchtauftragswalze von Druckwerken von Nassoffsetmaschinen steht, wobei der Walzenkörper aus Stahl, Aluminium oder kohlefaserverstärktem Kunststoffmaterial besteht, **gekennzeichnet durch** einen Überzug des Walzenkörpers aus hochverschleißfester Oxidkeramik oder aus verschleißarmem Hartmetall, in dessen Schichtmatrix zur Umfangsfläche des Walzenkörpers hin offene Poren ausgebildet sind und wobei die poröse Beschichtung eine Oberflächenrauhigkeit von R₂ von 5 µm bis 25 µm hat.

2. Verwendung wie in Anspruch 1 beansprucht, **dadurch gekennzeichnet, dass** der poröse Überzug aus Al₂O₃, Cr₂O₃, TiO₂, SiO₂ oder ZrO₂ oder aus Mischungen daraus besteht.

3. Verwendung wie in Anspruch 1 beansprucht, **dadurch gekennzeichnet, dass** der poröse Überzug aus WC/Co, Cr₃C₂/NiCr, NICrBSi, WC/Ni, TiC/Ni, Molybdän, Chrom oder aus Mischungen daraus besteht.

4. Verwendung wie in einem der vorhergehenden Ansprüchen beansprucht, **dadurch gekennzeichnet, dass** der poröse Überzug eine Dicke von 25 µm bis 2000 µm, vorzugsweise eine Dicke von ungefähr 150 µm aufweist.

## Revendications

1. Utilisation d'un corps à rouleaux pour la formation améliorée d'une émulsion encre-eau dans des unités d'impression de machines d'impression en offset à l'état humide, corps à rouleaux qui est en contact direct avec le rouleau de forme mouilleur des unités d'impression des machines d'impression offset à l'état humide, le corps à rouleaux étant constitué d'une matière plastique renforcée avec de l'acier, de l'aluminium ou des fibres de carbone, **caractérisée par** un revêtement du corps à rouleaux qui est constitué de matières céramiques à base d'oxydes hautement résistantes à l'usure ou d'un métal dur résistant à l'usure, des pores qui sont ouverts vers la surface circonférentielle du corps à rouleaux étant présents dans la matrice de la couche du revêtement, et le revêtement poreux ayant une rugosité de surface R_{z} de 5 µm à 25 µm.

2. Utilisation suivant la revendication 1, **caractérisée en ce que** le revêtement poreux consiste en Al₂O₃, Cr₂O₃, TiO₂, SiO₂ ou ZrO₂ ou leurs mélanges.

3. Utilisation suivant la revendication 1, **caractérisée en ce que** le revêtement poreux consiste en WC/Co, Cr₃C₂/NiCr, NiCrBSi, WC/Ni, TiC/Ni, molybdène, chrome ou leurs mélanges.

4. Utilisation suivant l'une quelconque des revendications précédentes, **caractérisée en ce que** le revêtement poreux a une épaisseur de 25 µm à 2000 µm, de préférence une épaisseur d'environ 150 µm.
